

Jan. 6, 1931.

C. H. BOYLES

1,788,146

RESISTANCE UNIT AND METHOD OF PRODUCING THE SAME

Filed April 30, 1928

201-63

Fig. 1.Fig. 2.Fig. 3.

INVENTOR.

Carroll H. Boyles.  
BY  
Morsell, Keeney & Morsell  
ATTORNEYS.

## UNITED STATES PATENT OFFICE

CARROLL H. BOYLES, OF MILWAUKEE, WISCONSIN

## RESISTANCE UNIT AND METHOD OF PRODUCING THE SAME

Application filed April 30, 1928. Serial No. 273,969.

This invention relates to improvements in resistance units and method of producing the same.

It is one of the objects of this invention to provide an improved resistance unit, which, when energized, will radiate heat of great intensity such as is necessary in smelting furnaces, electric stoves and heaters, electric irons, and the like.

10 It is a further object of this invention to provide a novel method of producing this improved resistance unit.

It is a further object of this invention to provide a resistance unit having an outer 15 coating of material which will prevent oxidation of the heating element within.

It is a further object of this invention to provide a resistance unit which is efficient in operation, simple in construction, and well 20 adapted for the purpose described.

With the above and other objects in view, the invention consists of the improved resistance unit and method of producing the same, and all its parts and combinations as 25 set forth in the claims, and all equivalents thereof.

In the accompanying drawing in which the same reference characters designate the same parts in all of the views:

30 Fig. 1 is a longitudinal sectional view of the improved resistance unit;

Fig. 2 is a sectional view taken on the line 2-2 of Fig. 1; and

Fig. 3 is an end view thereof.

35 Referring to the drawing, the numeral 5 designates the heating element which is composed of a portion of gas carbon or amorphous carbon mixed with a portion of carbide of boron, the latter substance being thoroughly pulverized. These two ingredients

40 are then mixed with a binding material such as coal tar or sodium silicate, and the compound is molded into the desired form, preferably the form shown. The molded product is next subjected to a high hydraulic pressure to render it as dense as possible, and is then heated to a temperature of 1200° F. to 1400° F. for a period of 24 to 48 hours to expel all volatile compounds. The exact proportions

50 of the various ingredients used may be

varied in accordance with the resistance desired in the unit. The following is the formula used:

46% to 80% carbon, 52% to 12% carbide of boron, 2% to 8% sodium silicate. 55

Pulverized corundum may be substituted for the carbide of boron, and in the claims it is to be considered as the full equivalent of the latter substance.

The numeral 6 in the drawing designates 60 the outer covering which is a non-conductor of electricity, and which prevents air from reaching the heating element within and oxidizing the latter. This outer coating is formed by mixing a quantity of pulverized 65 corundum with a suitable binder such as sodium silicate. The following proportions may be used:

85% to 98% corundum, 15% to 2% sodium silicate. 70

This formula may be varied by substituting pulverized carbide of boron for the corundum. The carbide of boron is to be considered as the full equivalent of corundum in the claims. 75

After this compound has been prepared it is molded around the heating element and is subjected to a high pressure. The unit is then subjected to a temperature of 1800° to 2000° F. for a period of 18 to 36 hours to expel all remaining volatile compounds and to harden the unit. 80

The end portions 7 of the unit are preferably composed of a material having a low resistance to more readily conduct electricity. 85 If desired, this may be accomplished by coating the ends of the heating element with a conductor material such as copper, or the ends may be formed entirely of such material.

The ends 7 are of larger diameter than the heating element proper and are molded with it to form a spool-shaped core for the outer coating.

90 From the foregoing description it may be seen that the improved resistance unit is simple in construction, efficient, and well adapted for the purpose described.

What I claim is:

1. As a new article of manufacture, a re- 100

5 sistance unit comprising an inner heating element composed of 46-80% carbon, 52-12% carbide of boron and 2-8% binder, and an outer covering for a portion of the same composed of 85-98% corundum and 15-2% binder.

10 2. As a new article of manufacture, a resistance unit comprising an inner heating element composed of 46-80% carbon, 52-12% carbide of boron, and 2-8% sodium silicate, and an outer covering for a portion of the same composed of 85-98% corundum and 15-2% sodium silicate.

15 3. The method of producing a resistance unit consisting of mixing together carbon, carbide of boron, and a binder, molding the same into a desired form, subjecting the compound to the action of pressure and heat, mixing a second compound of corundum and a 20 binder, molding this compound around the first compound, and subjecting the product to pressure and heat.

25 4. The method of producing a resistance unit consisting of mixing together 46-80% carbon, 52-12% carbide of boron, and 2-8% binder, molding the mixture into a desired form, subjecting the compound to the action of pressure and heat, mixing a second compound of 85-98% corundum and 15-2% 30 binder, molding this compound around the first compound, and subjecting the product to the action of pressure and heat.

35 5. The method of producing a resistance unit consisting of mixing together 46-80% carbon, 52-12% carbide of boron, and 2-8% sodium silicate, molding the mixture into a desired form, subjecting the compound to the action of pressure and heat, mixing a second compound of 85-98% corundum and 40 15-2% sodium silicate, molding this compound around the first compound, and subjecting the product to the action of pressure and heat.

45 6. The method of producing a resistance unit consisting of mixing together 46-80% carbon, 52-12% pulverized carbide of boron, and 2-8% sodium silicate, molding the mixture into a desired form, subjecting the mixture to a high pressure, heating the mixture 50 to a temperature of 1200°-1400° F. for 24-48 hours, mixing a second compound of 85-98% corundum and 15-2% sodium silicate, molding this compound around the first compound, subjecting the product to a high pressure, and heating the product to 1800°-2000° 55 F. for 18-36 hours.

60 7. As a new article of manufacture, a resistance unit comprising an inner heating element composed of approximately 63% carbon, 32% carbide of boron, and 5% binder, and an outer covering for a portion of the same composed of approximately 91½% corundum and 8½% binder.

65 8. As a new article of manufacture, a resistance unit comprising an inner heating ele-

70 ment composed of 46-80% carbon, 52-12% carbide of boron, and 2-8% binder, and an outer covering for a portion of the same composed of an electrical insulating material which will protect the inner heating element from oxidation.

75 In testimony whereof, I affix my signature  
CARROLL H. BOYLES.

80

85

90

95

100

105

110

115

120

125

130